

## UNITED STATES PATENT OFFICE

ERNEST E. NOVOTNY, OF PHILADELPHIA, PENNSYLVANIA

## STENCIL SHEET

No Drawing.

Application filed July 11, 1928. Serial No. 292,023.

This invention relates to the production of a type or stylus impressible stencil sheet of improved composition, and to an improved method of making the same. Broadly the object of the invention is to utilize the film forming properties of carbohydrate esters softened or modified in a new and novel manner.

At least one of the softening or modifying agents are acid free bodies of a very staple nature and which therefore do not disintegrate the carbohydrate ester; nor do these bodies, themselves, decompose because of oxidation or become rancid.

At least one of the softening or modifying agents is preferably an absorbent of the other, thus preventing the sweating out of the liquid softening agents. This relatively dry absorbent also makes dispersion of the modifying agents in the cementitious mass more thorough and uniform. This and the use of a colloid mill or a high speed mechanical stirring device so subdivides the softening or modifying bodies and the cementitious mass that the resulting stencil sheet is very pliable and soft and yet of great tensile strength.

My stencil sheets have long keeping qualities and may be made and kept in a preferred condition for ready use without previous treatment. They are neither sticky nor tacky and they may be relied upon to cut easily and sharply with uniform visibility. When written upon, my stencil sheets produce an inklike impression on the backing sheet which may be easily read.

The prior art shows the use of various carbohydrate esters as the cementitious material in the making of the dry lacquer type of stencil sheets. These cementitious esters are usually the nitroderivatives of cellulose (pyroxylan), or the acetic derivatives of cellulose, starch, sugar, and various vegetable gums.

The effective modifying or softening agents are usually vegetable oils, fats, and fatty acids. These oils, fats and fatty acids tend to oxidize after a time, especially when in thin films as in a stencil sheet, and these products become odorous and rancid. The oxidization of the oils changes these to fatty acids. Most of the commercial grades of oils such as are used in stencil sheets, as for example, castor

or palm oils contain quantities of free fatty acids when purchased.

It is well known that acids greatly affect the stability of the nitrocellulose, causing disintegration. While this effect is more pronounced with strong acids which cause comparatively rapid disintegration with the liberation of oxides of nitrogen, even such weak acids as oleic acid bring about this change over a period of time. These disintegration products of nitrocellulose in turn react upon an acid such as oleic, causing it to rapidly become rancid. The result is that where a fatty acid is present in a stencil sheet and this also applies particularly to oleic acid the sheet becomes sticky, tacky, soft, and unfit for use in a comparatively short time, furthermore, dyes which are often used in a stencil sheet, to make the writing or ornamentation visible, are bleached by these disintegration products.

My modifying agents contain no free acids and in fact the sodium or potassium soaps are mildly alkaline and therefore act to stabilize the nitrocellulose, thus producing a sheet which can be kept for a longer period of time than has heretofore been possible.

To refer again to the prior art, it will be noted that various preservatives have been suggested but the fact remains that the acids present do the harm. Actual tests have proven that these preservatives cannot prevent the disintegration of the nitrocellulose film so long as these acid bodies are present nor can the preservatives prevent the oxidization of fats and oils when in thin films as in a stencil sheet. As a matter of fact, all of the dry lacquer stencils on the open market at present, known to me, are of the nitrocellulose type containing large quantities of fatty acids.

In the volumes of prior art examined, no stress is made of the need for uniform and thorough dispersion of the modifying material within the cementitious body. This is of great importance and it may be stated that with the same initial ingredients and proportions relatively useless stencils may be made because of poor dispersion in the starting materials, and, on the other hand, exceptional results may be had if properly combined,

Thorough dispersion reduces the size of the colloidal particles, thus increasing the surface within the mass and decreasing the thickness of the internal cementitious film. A 5 strong stencil sheet results which is easily and sharply impenetrable with the desired ornamentation without preliminary preparation of the stencil coating. Dispersion to the most thorough degree will often permit the 10 use of modifying agents ordinarily not suitable because of sweating out of the film, resulting in sticky and tacky stencil surfaces which clog the type and otherwise are the cause of much annoyance.

15 A relatively soft variety of cementitious material may be made into a stencil sheet which will cut fairly well when modified with air or gas bubbles thoroughly dispersed therein. This results in the mass of material 20 being broken up into films of infinite thinness which lack toughness. A stencil sheet coated with this composition will be easily impenetrable.

25 After prolonged experimentation I have found that a stencil sheet can be made which will be very uniform in quality even when made in large commercial quantities and which will have long keeping qualities.

30 Stable modifying agents which do not disintegrate the nitrocellulose film are of first importance. My preference is for the use of an alkyl ester of oleic acid such as for example ethyl, methyl, or butyl oleate. These alkyl esters of oleic acid can be readily 35 made, have a very desirable softening effect on the cementitious film, are very clear transparent bodies having high boiling points and do not evaporate from the stencil coating. These esters will not spoil or become 40 rancid nor will they promote the disintegration of the cementitious material of the stencil. These stencils may therefore be kept in stock in ready to use condition for a long period of time.

45 The alkyl esters of a fatty acid are in themselves not sufficient to produce an ideal stencil sheet. If sufficiently large quantities are incorporated these materials sweat out to the surface and make a stencil disagreeable 50 and objectionable to handle. The use of an absorbent is desirable and an absorbent such as will also tend to soften the cementitious film is preferably used. Thus I produce and maintain a satisfactory condition of plasticity, and a dry surface film free from stickiness. This absorbent should also promote 55 intimate and uniform dispersion. The material should also be stable and have long keeping qualities in the stencil film and should not cause the disintegration of the nitrocellulose.

60 I have found that the metallic soaps and more especially the metallic soaps of fatty acids to be most suitable for this purpose. 65 Preferably I use the dry and substantially

pure soaps having only traces of free alkali. While the potassium soaps give products of a softer nature, the sodium soaps on the other hand promote better dispersion and are more absorbent for my purpose.

70 Of the fats and fatty acids the soaps of most any of these will give results, but the potassium or sodium laureate or oleate are to be preferred.

I prefer to use sodium oleate because this 75 material is cheap and provides the necessary softening, absorbent, and dispersion qualities when used with my preferred choice of alkyl ester of oleic acid, i. e., ethyl oleate.

I find that the use of an alkyl ester of 80 oleic acid alone without the use of a metallic soap of a fatty acid produces an inferior stencil sheet and as both products are stable, and inexpensive, and as the soap tends to stabilize the nitrocellulose film I find it highly desirable to use this combination of compounds.

I may also use a wax preferably of vegetable origin such as carnauba wax which is previously dissolved in a suitable solvent such as alcohol or ether. Instead of dissolving the wax I find that a better result is attained by using a diluent such as toluol which will when heated with the wax produce a soft modification. This heated wax solution or 90 mixture is added while hot to the other ingredients and thoroughly beaten or dispersed therein. Other waxes can be used but those that do not form fatty acids are to be preferred. The addition of a small quantity 95 of this waxy material helps to promote dispersion and to maintain a dry surface free from stickiness. While the use of the wax is not necessary, it is more simple to maintain a soft but dry surface film when it is 100 used.

Rapid and thorough mechanical agitation is necessary for the reasons before stated and because the substantially dry sodium oleate will not be properly dispersed otherwise. It 110 is probable that the difficulty encountered in endeavoring to introduce this material into a pyroxylin lacquer solution brings about the thorough, minute, and colloidal dispersion of the modifying agents within the cementitious film when rapidly and thoroughly beaten into the mass. Because of the thorough dispersion and the absorbent effect of the relatively moisture free soap, the ethyl oleate is retained in the stencil sheet.

115 The use of these modifying materials, the alkyl esters of oleic acid and the metallic soaps of fatty acids and the use of these in combination with each other is the most particular improvement I have disclosed in this application.

120 While the use of various carbohydrate esters with the above modifying agents is possible, I do not find any cementitious ma- 130

terial of this type as suitable for my purpose as nitrocellulose (pyroxylin).

It should also be noted that the modifiers described herein are not commonly considered as oily substances but are stable derivatives of fatty acid substances.

In carrying out my invention, the following formula of my preferred form of stencil composition is given.

10 If it is desired to purchase a lacquer solution from the lacquer manufacturer, procure a clear lacquer, preferably resin free, containing from 8 to 12 parts of 15 to 20 second nitrocellulose (pyroxylin) and 92 to 15 88 parts respectively of suitable solvents and diluents.

The lacquer manufacturer can also supply a suitable thinner and about one half the quantity of this by weight of the lacquer will be needed.

20 I, however, prefer to cut my own lacquer because it is then more readily possible to control the product to the viscosity and percentage of solid nitrocellulose content. The 25 materials needed are given and the parts are by weight throughout.

Pyroxylin (nitrocellulose) 15 to 20 sec. Parts  
(moist) ----- 570  
Toluol ----- 800  
30 Butanol ----- 1100  
Ethyl alcohol ----- 1100  
Butyl acetate ----- 2750

The pyroxylin and toluol are placed into a 35 suitable stirring device and the mass is thoroughly and uniformly wetted with the toluol to prepare the nitrated cotton for the action of the solvents. Preferably I add the other ingredients while stirring continuously until 40 a perfect solution is obtained. This material may be stored in drums for use as required. The purchased lacquer solution may be substituted for the above solution. This cementitious mixture will hereafter be referred to 45 as pyroxylin lacquer.

The next step is to introduce the modifying agents, color and further pyroxylin lacquer thinners to produce a colloidal mass properly tempered and dispersed for use as a stencil 50 coating material.

I preferably provide a mechanical stirring device of relatively high speed or I may use a colloid mill. The object being to thoroughly incorporate the ingredients together and to minutely disperse the modifying agents within the cementitious mass.

Two formulæ are given. No. 1 includes the use of carnauba wax while No. 2 omits this ingredient. The proportions given are by 60 weight and are those I preferably use but should be considered as illustrative examples only. The carnauba wax is given as dry weight of wax although it is introduced hot with the toluol used to cut it with. I use ordinarily 1 part of carnauba wax and 48

parts of toluol heated on a hot plate and add hot. Some of the toluol is lost in heating unless a reflux condenser is used, although I do not find the condenser necessary.

|                                                            | No. 1 | No. 2 | 70 |
|------------------------------------------------------------|-------|-------|----|
| Pyroxylin lacquer.                                         | 96    | 96    |    |
| Ethyl oleate.                                              | 48    | 48    |    |
| Sodium oleate, dry.                                        | 5     | 12    |    |
| Carnauba wax.                                              | 1     |       |    |
| Toluol.                                                    | 48    |       | 75 |
| Victoria blue B dye.                                       | q.s.  | q.s.  |    |
| Stir rapidly for 15 minutes and thin with lacquer thinner. | 48    | 48    |    |

Stir some more.

The mixture is now ready to be poured into the coating pan where the yoshino paper or other porous paper or fabric may be coated, impregnated or sprayed with the material and the excess, if impregnated, removed in any suitable manner as by scraping the sheet over a wire or straight edge.

If viscosity of solution is too thick, more lacquer thinner can be used and likewise if a heavier stencil sheet is desired either a thicker sheet of stencil material should be used or the quantity of lacquer thinner may be reduced.

By carefully controlling the viscosity of the pyroxylin lacquer by the addition of suitable quantities of say  $\frac{1}{2}$  second pyroxylin and making viscosity determinations any material un-uniformity in the stencil product will be avoided.

The solvents and diluents given for the production of the pyroxylin lacquer can be used in the proportions given for the lacquer thinner. The commercial lacquer thinner is less expensive as it is higher in inexpensive diluents.

It will be noted that the lacquer formula I have given need not contain any nitrocellulose plasticizers such as dibutyl phthalate, diamyl phthalate, tricresyl phosphate, etc. These are ordinarily used to soften or weaken the lacquer film itself because the modifying agents are insufficient for this purpose and also to prevent the crystallization of the modifiers within the lacquer film. Various oils, fats and fatty acids combined with nitrocellulose films often crystallize in this manner and make the use of these high boiling mutual solvents necessary. These plasticizers often sweat out, making the surfaces sticky and make the dispersion of the modifying agents more difficult.

A lacquer thinner formula such as is most suitable is given below. Proportions are by weight.

|                                   |     |     |
|-----------------------------------|-----|-----|
| Toluol -----                      | 65  | 125 |
| Benzol -----                      | 50  |     |
| Amyl acetate -----                | 15  |     |
| Butyl acetate -----               | 85  |     |
| Ethyl acetate -----               | 100 |     |
| Ethyl alcohol (C. D. No. 1) ----- | 50  | 130 |

The formulæ and method need not be followed precisely as wide variations and departures are possible without material change in the technical effect. The pyroxylin lacquer can be substituted for by the use of other carbohydrate esters when used under changed conditions of solvents, etc. The use of other solvents and diluents and other proportions is possible.

10 The production of the alkyl ester of oleic acid is well known. The sodium or potassium oleate may be readily purchased at any general chemical supply source.

15 When the stencil sheet is first coated and Victoria blue B is used as the dye, the stencil will be almost black in color. As soon as the solvents dry out (which takes only a few minutes) the product becomes a beautiful transparent and uniformly colored sheet free 20 from the cloudy semi-transparent appearance of stencils made of pyroxylin lacquer including various fats, oils, fatty acids, etc.

25 The coating is easily removed and the portion so removed produces an inklike copy of the ornamentation produced thereon, thus greatly facilitating the proof reading of the work. By supplying a white lithocoated backing board this result is greatly enhanced.

30 The coating mixture produces films very easily displaced and, therefore, for an inexpensive stencil sheet ordinary porous paper coated with this mixture on one or both faces can be used. The results are not 35 so good as where yoshino paper is used, but for autographic work it is more easily written upon and there is an advantage in cost where a large number of stencils are needed to replace other method of duplication as by 40 the gelatine copy method.

45 Where a reproduction of an electrotype, etching or body of type is desired, if this relieve block or body be heated the stencil material may be easily displaced with comparatively little pressure.

50 The ethyl oleate has a pleasant, fruity, apple like odor, which is very penetrating however, and this can be changed by the addition of a desired perfume such as oil of wintergreen.

55 Although a preservative is not necessary, however if desired because of the use of crude materials or for other precautions, a small quantity of thymol or resorcinol can be used, quantity by weight about .01% of the weight of the entire coating material treated.

What I claim is—

1. An impressible stencil sheet having a porous base and a coating including a cellulose ester and ethyl oleate.
2. An impressible stencil sheet having a porous base and a coating including a cellulose ester, an alkyl ester of oleic acid and 65 a wax.

3. An impressible stencil sheet having a porous base and a coating including a cellulose ester, ethyl oleate and carnauba wax.

4. An impressible stencil sheet having a porous base and a coating including nitrocellulose, an alkyl ester of oleic acid and a wax.

5. An impressible stencil sheet having a porous base and a coating including nitrocellulose and an alkyl ester of oleic acid.

Signed at Philadelphia in the county of Philadelphia and State of Pennsylvania this 9th day of July A. D. 1928.

ERNEST E. NOVOTNY.

80

85

90

95

100

105

110

115

120

125

130

70

75

80

85

90

95

100

105

115